

## UNITED STATES PATENT OFFICE

ALBERT C. FISCHER, OF CHICAGO, ILLINOIS, ASSIGNOR TO THE PHILIP CAREY MANUFACTURING COMPANY, A CORPORATION OF OHIO

## CONSTRUCTIONAL MATERIAL

No Drawing.

Application filed August 15, 1927. Serial No. 213,188.

This invention relates to constructional material, such as, roofing material, insulating material, tapes, shingles, packing and the like.

5 The object of my present invention is to provide such constructional materials with an adhesive coating which is normally sticky or tacky to the touch and which lastingly maintains this mastic condition whereby the material may be packed and stored for long 10 periods of time without losing its tackiness and may be transported to its place of installation and used in such tacky condition without further treatment.

15 A further object of my invention resides in the application of this normally lastingly adhesive, sticky to the touch, to sheets or strips of carrier material, hereinafter called vehicles, so that when rolled into package 20 form or placed face to face in contact with a similar sheet for packing and storing and transportation, they may be unrolled or pulled apart readily without tearing or damaging, and can be installed in tacky condition; in this instance the tacky coating permits the facile separation of the contacting 25 vehicle surfaces, the line of cleavage passing through the mastic itself. The vehicle thus provided with a lasting adhesive, mastic 30 coating is particularly adapted to act as a packing for various types of installations, not only because of the waterproofing quality of the mastic but also because of its pronounced and lasting quality of adhesiveness 35 and further because of its plasticity.

A further object of my invention resides in providing a constructional material which includes a vehicle saturated with a bituminous adhesive, such saturant being treated 40 with an overcoating of a viscous adhesive, which will be separable along the lines of such coating, whereby the vehicles when so coated may be separable from objects to which they adhere or from similar vehicles.

45 In the present invention the vehicle may consist of sheets, strips, or slabs of tar paper, felt, fabric, fibers or other preferred material.

This saturant may also be a single vegetable or bituminous adhesive, such as, cot-

tonseed, Foot's pitch or road oil, sludges and semi-liquid, bituminous substances of varying consistencies, such saturants, when treated with an overcoating of a viscous vegetable or combination vegetable and bituminous adhesive will be separable along the lines of such coating.

The coating with which the vehicle is thus saturated on either one or both sides preferably comprises a slow-drying, tacky, bituminous, vegetable or animal adhesive or combination of two or more, which approximates the following specifications, or may be more or less fluid.

(1) The consistency at 77° F. should be 65 below 7.0.

(2) The susceptibility factor should be as low as possible, preferably under 25.

(3) The ductility at 77° F. should be as high as possible and preferably over 25 centimeters.

(4) Fusing point by K and S method should be between 80° and 100° F.

(5) It should appear tacky and adhesive at normal temperature and retain this property as long as possible on exposure to air.

This formula is merely a standard and other formulas more or less fluid may be used with or without a suitable filler as a flow retarder, or the flow tendency may be stopped 80 by using a non-flowing gummy substance in combination.

It will be understood that my invention contemplates constructional material, the adhesiveness of which serves to hold said material in place in distinction to other materials which involve the use of pitch, or other material, mopped on at the time of assembling the material. This is especially true in the application of the invention to roofing sheets, 90 for the purpose of holding the sheets of roofing material in place. It will be understood that after two sheets of building material according to the present invention have been separated, the adhesive surface of one sheet 95 will be placed in contact with the non-adhesive surface of another sheet. The adhesive or mastic will cause a union with non-adhesive surfaces to which it is applied, which union may be made very excellent by means 100

of rolling and which will improve in the course of time.

It will also be understood that if it should be found that the adhesive surface of a sheet should become dried out, a solvent such as toluol, benzol, kerosene, or cotton oil, may be used to bring the sheet back into adhesive state.

The subject matter of this application has 10 been withdrawn from my prior Patent No. 1,550,310, issued August 18, 1925.

I claim:

1. Constructional material comprising a vehicle saturated with a road oil of bituminous nature, and coated with a normally viscous bituminous adhesive which is separable along the lines of such coating from contact with another sheet.
2. Constructional material comprising a vehicle saturated with a semi-liquid bituminous substance and coated with a normally viscous bituminous adhesive which is adapted to be separated along the lines of such coating from contact with another sheet.
3. Constructional material comprising a vehicle saturated with a bituminous adhesive and treated with an overcoating of normally viscous adhesive, separable along the lines of such coating from contact with another sheet.

Signed at Chicago, Illinois, this 9th day of August, 1927.

ALBERT C. FISCHER.

35

40

45

50